

# UNITED STATES PATENT OFFICE.

WILLIAM VIRGO WILSON, OF JUBILEE STREET, MILE END, COUNTY OF MIDDLESEX, ENGLAND.

## MANUFACTURE OF MATERIAL FOR ELECTRIC INSULATION.

SPECIFICATION forming part of Letters Patent No. 294,557, dated March 4, 1884.

Application filed January 4, 1884. (No specimens.) Patented in England July 11, 1883, No. 3,413.

*To all whom it may concern:*

Be it known that I, WILLIAM VIRGO WILSON, a subject of the Queen of Great Britain, residing at Jubilee Street, Mile End, in the county of Middlesex, England, color-manufacturer, have invented certain new and useful Improvements in the Manufacture of Material for Electric Insulation, (for which I have received Letters Patent in Great Britain, No. 3,413, dated July 11, 1883,) of which the following is a specification.

This invention has for its object the consolidation of wood or vegetable tar by means of nitro-cellulose, the nitration of which has not been carried beyond the point which will effect its greatest solubility—a modification of this body quite well understood. Both these before-mentioned substances are well known to have considerable non-conducting properties, and when properly incorporated by the intervention of some of the solvents of nitro-cellulose—such as methylic alcohol or ethylic alcohol and mineral naphtha, or other well-known solvents—the resulting compound possesses very high insulating power.

In practice I take two hundred parts of the tar above named and raise its temperature to about 200° Fahrenheit, and I then add one hundred parts of the nitro-cellulose prepared as above described and softened by one or more of the solvents to which allusion has been already made by a now well-ascertained process. Although I have found the above proportions and temperature advantageous, I do not confine myself to them. The mixture I then thoroughly incorporate and transfer to

a masticating or grinding machine—by preference to the latter—constructed in a similar manner to machines now in operation for the trituration of gutta-percha and india-rubber. 40 When the mass in the machine has become homogeneous, it is ready for application to the purpose of insulation in all its branches, and I use this mixture for insulating electric conductors by means of the ordinary covering 45 machinery now employed for such purposes in a manner well understood. This mixture I apply in its present condition, or I further mix or compound it with one or more of the following substances, such as barium sulphate, chalk, talc, calcium sulphate, alumina, magnesia, oxide zinc, silica, &c., whereby the mixture is rendered cheaper and its combustibility reduced. These may be mixed during any stage of the manufacture; but I prefer to 55 incorporate them while the mass of material is in the masticating or grinding machine.

Having thus described the nature of my invention and the manner of performing the same, I would have it understood that what I claim is—

The consolidation of wood or vegetable tar by the use of nitro-cellulose softened as hereinbefore set forth, and its application to the purpose of insulating electric conducting- 65 wires.

WILLIAM VIRGO WILSON.

Witnesses:

T. W. KENNARD,  
53 Chancery Lane, London.  
JNO. DEAN,  
17 Gracechurch St., London.